

June 14, 1960

G. F. TISINAI ET AL

2,940,879

PRODUCTION OF AUSTENITIC STEEL ALLOYS

Filed Dec. 29, 1955



INVENTORS:

BY  
James K. Stanley  
George F. Tisina  
Carl H. Samans  
Arthur G. Gilkes  
ATTORNEY

**1**

2,940,879

**PRODUCTION OF AUSTENITIC STEEL ALLOYS**

George F. Tisinai, Highland, Ind., and James K. Stanley and Carl H. Samans, Chicago, Ill., assignors to Standard Oil Company, Chicago, Ill., a corporation of Indiana

Filed Dec. 29, 1955, Ser. No. 556,214

1 Claim. (Cl. 148—3)

Our invention relates to means for the production of stable austenitic stainless steels without depending upon nickel as an essential alloying element. More particularly, it relates to the production of austenitic stainless steels by an economically attractive melting process.

The chrome alloy stainless steels are normally ferritic or martensitic in structure. Although austenitic iron-chromium-nickel and iron-manganese-carbon alloys are well known, so far as we know, it has not been possible to produce completely austenitic steels without the use of nickel or manganese. These alloys have useful, distinctive properties including a high degree of oxidation and corrosion resistance but their cost and the strategic significance of nickel and manganese have stimulated a great deal of research by investigators, both here and abroad, in an effort to produce austenitic alloys by other means.

The iron-chromium-carbon system, for example, has been studied extensively. Ordinarily carbon-free iron-chromium alloys containing more than 13% chromium are ferritic at all temperatures. Below 13% chromium the austenitic field exists above 1550° F. Carbon additions will expand the austenite field up to about 21% chromium at temperatures above 1550° F. With increased chromium content above 21%, the single phase austenite field is eliminated. Krivobok and Grossman, Trans. Am. Soc. Steel Treat., v. 18 (1930), pp. 760-807, have reported production of an essentially austenitic structure in a steel containing as high as 21% chromium by addition of 0.62% carbon. On the other hand, their work with 28% and 33% chromium alloys of variable carbon content (up to 0.70%) resulted in only minor amounts of austenite.

The effect of nitrogen on the structure of iron and chromium alloys also has been extensively investigated. The most significant work appears to be that of Colbeck and Garner, J. Iron and Steel Inst., v. 193 (1939), pp. 99-135, who have reported the production of 24% chromium alloys containing as much as 60% austenite and of 27% chromium alloys containing as much as 50% austenite. See also B. G. Bandel, Archiv. f. d. Eisenhuttenwesen, vol. 11, pp. 139-144, 1937, wherein the partial austenitization of a number of chromium alloys by addition of nitrogen is reported. A completely austenitic structure, however, has not been realized for high chromium alloys, insofar as we are aware, except for the single non-reproducible example reported by Krivobok and Grossman, *supra*, without the use of upwards of about 4% nickel.

Recently, however, as described in co-pending application of Tisinai and Stanley, Serial Number 525,275, filed July 29, 1955, now Patent No. 2,890,995, granted June 16, 1959, essentially austenitic alloys containing up-

**2**

wards of 21% chromium have been produced. The new products followed the discovery that a critical relationship exists between carbon and nitrogen affecting austenitization, a relationship which prior investigators appear to have overlooked, perhaps because of the unexpectedness of any cooperation between these minor constituents in this respect or perhaps because of the confusing fact that nearly all steels contain some concentration of carbon as a constituent impurity. The amount of nitrogen that can be retained by the higher chromium alloys is increased tremendously when the alloys contain up to about 1% carbon, and completely austenitic alloys can be produced when the proportions of carbon and nitrogen are adjusted to a critical relationship for a particular chromium content, apparently through some synergistic action. A hyperbolic relationship exists between carbon and nitrogen in the chromium alloy steels which appears to be responsible for stabilization of an austenitic structure. The higher the carbon content, the lower is the nitrogen content necessary to make the resulting alloy completely austenitic. Conversely, the lower the carbon content, the higher is the amount of nitrogen that is required to make the alloy completely austenitic. As the amount of chromium in the alloy is increased, larger amounts of carbon and nitrogen appear to be required for a stable austenitic structure. At the higher chromium contents, e.g. say 27 to 33% chromium, the stable austenite field becomes smaller although useful alloys of stable austenitic structure containing coexisting chromium carbide may be formed over a field of broader range.

The new iron-chromium-carbon-nitrogen alloys have valuable corrosion-resistant properties, including oxidation resistance at elevated temperatures at least up to 900° F. and also above 2000° F., of a type associated with austenitic nickel- and manganese-containing chrome alloys. In other respects, however, the new austenitic alloys appear to be quite distinctive in properties such as tensile and yield strength, work-hardening and the like.

Although the relationship between carbon and nitrogen appears to have some general application to chrome alloy steels, alloys of less than about 21% chromium content appear to lack the distinctive corrosion resistance and high structural stability of the new alloys. For example, a 21% chromium steel, even though of substantially austenitic structure, is borderline in oxidation resistance at 2000° F. Also, with chromium contents substantially above 33%, impractically high nitrogen contents are required to avoid restriction of the austenite field to the vanishing point although the two phase field of austenite plus carbide may have general usefulness.

The addition of nitrogen to conventional low-carbon, chromium-iron alloys however gives considerable difficulty in conventional casting. If more nitrogen than about  $\frac{1}{75}$  to  $\frac{1}{100}$  of the chromium content is added, gassy ingots result during solidification due to the loss of a considerable amount of the nitrogen introduced. We have found, however, that when the carbon content of the melt is sufficiently high, e.g. about 0.2% and advantageously from 0.3 up to about 1%, loss of nitrogen is minimized, or entirely prevented, so that high nitrogen alloys containing up to as much as 1% nitrogen can be cast directly. When the composition of a molten iron-chromium alloy is properly controlled, it solidifies in the completely austenitic state rather than in the expected ferritic state. Moreover, the high nitrogen is apparently

retained in solid solution without giving rise to excessive porosity, produced by evolving nitrogen, as in the case of ferritic ingots. Alloys can be produced in good quality with a completely austenitic structure at room temperatures. In casting, the retention of sufficient nitrogen in alloys containing less than about 0.3% carbon may be difficult when operating at atmospheric pressure but can be simplified by use of pressure casting techniques. Cast ingots of completely austenitic structure can be satisfactorily reduced in size by forging.

Thus, by the present invention, essentially completely austenitic, high chromium stainless steel alloys can be produced by forming a melt comprising iron, about 21 to 33% chromium, about 0.20 to 1.0% carbon and sufficient nitrogen added in the form of a stable combination with a metal which is fusible in the range of about 2000° to 2400° F., casting the resulting melt and rapidly cooling the cast product to a temperature below about 800° F. The process affords substantial advantages in production, economy and output compared to the use of nitrogenization or powder metallurgy techniques for producing the austenitic alloys.

The cast alloy is cooled from about 2200° F. to below about 800° to 900° F. rapidly enough, as by quenching, to prevent transformation of the austenitic structure to the ferritic structure. Although the change in structure from austenitic to ferritic is sluggish, some decomposition of austenite may occur on slow cooling as by air cooling of large sections. Quenching or rapid cooling therefore is desirable. A partially decomposed austenite, however, can be converted to an all austenite structure by reheating to about 2000° to 2400° F., preferably 2200° F., followed by rapid cooling to below 800° F. Also, although the austenitic grain size may be quite large in the cast alloys, it can be refined for control of mechanical properties by decomposing the alloys to ferrite, carbides and nitrides by heating to temperatures within the range of about 900 to 1300° F. followed by reaustenitizing for short periods of time at 2200° to 2300° F.

The materials used are charged in the usual way to a suitable melting furnace. A technical grade of iron or carbon steel, rather than pure iron, is used since the customary steel-making impurities appear to exert a beneficial stabilizing effect. The source of chromium, advantageously, is a commercial ferrochrome although the metal itself can be used. The source of carbon may be the steel or the ferrochrome, supplemented by the addition of graphite or a metal carbide. Nitrogen advantageously is supplied by use of a high nitrogen ferrochrome. For example, nitrogen ferrochromes of from  $\frac{3}{4}$  to 2% nitrogen in  $\frac{1}{2}$  % steps containing 0.1% carbon and about 70% chromium are available. Metal nitrides such as the chromium nitrides, CrN and particularly Cr<sub>2</sub>N, the iron nitrides Fe<sub>2</sub>N, Fe<sub>3</sub>N and Fe<sub>4</sub>N, silicon nitride Si<sub>3</sub>N<sub>4</sub>, and the like also have value. Other ferrochromes are available as sources of nitrogen and carbon, for example, 3 to 6% carbon ferrochromes of less than 0.025% nitrogen and 0.02 to 2.00% carbon ferrochromes of 0.5-0.75% nitrogen.

In the broader aspects of the invention, completely austenitic alloys can be produced with chromium contents in the range of about 21 to 33% by using selected proportions of carbon and nitrogen in the respective ranges of 0.1 to 1.0% and 0.2 to 1.0%. The resulting alloys may be pure, but as in conventional alloy production, they normally contain minor or non-detrimental amounts of constituent elements such as sulfur, phosphorus, manganese and silicon.

In the practice of the invention, we prefer to use a carbon content in the range of about 0.3 to 1.0%, more desirably 0.5 to 1.0%. The austenitic structure then is provided by using sufficient nitrogen in the range of about 0.3 to 1%, and with higher chromium contents, above about 0.5%. The resulting alloys appear to show

greater corrosion resistance, particularly with chromium contents in the range of about 24 to 30%. Also, nitrogen appears to be more effective than carbon in imparting improvement in tensile and yield strength properties.

The accompanying drawing illustrates application of the invention by reference to a simplified representation of a quaternary phase diagram which was based on the preparation and analysis of numerous samples of iron-chromium-carbon-nitrogen alloys.

10 The drawing illustrates the approximate limits of the austenite field in the iron-chromium-carbon-nitrogen system for four different chromium levels. Each panel represents a constant chromium content, the ordinates are percent nitrogen and the abscissas are percent carbon. 15 The diagram applies to alloys cooled rapidly from above 2200° F. All of the alloys above the curved lines are ferrite free, while the alloys below the curved lines contain ferrite. Thus, the drawing indicates the boundaries between the combined austenite ( $\gamma$ ) and the austenite plus carbide ( $\gamma+c$ ) fields, above the lines, and the combined austenite plus ferrite ( $\gamma+\alpha$ ) and austenite plus ferrite plus carbide ( $\gamma+\alpha+c$ ) fields, below the lines. It will be noted that the boundaries resemble the hyperbolic form; i.e. a hyperbolic relation appears to exist between the content of carbon and nitrogen which is responsible for the stable austenitic structure. The hyperbolic boundary shifts upward systematically as the chromium content is increased so that greater amounts of carbon and nitrogen are required to obtain the austenitic structure. Thus, from the 3-dimensional diagram of the drawing it may be seen that a curved surface exists which separates the upper austenitic field from austenite containing ferrite. Although alloys in the austenite plus ferrite field having a predominantly austenitic structure 20 may have engineering usefulness, the presence of more than about 15 to 20% ferrite will result in the loss of high strength and the loss of the non-magnetic nature, and possibly in the loss of general corrosion resistance commonly considered characteristic of the austenitic structure. The presence of small amounts of ferrite however 25 may lower the susceptibility of the austenite toward intergranular brittleness, may favor the resistance of the alloy to corrosion under stress, and may be useful to prevent weld cracking in the event the alloys are welded.

30 The invention will be further illustrated by reference to specific examples of alloys prepared according to the invention.

The steels used were charged from either "Armco Iron" or billet slabs obtained from a "1030" carbon 35 steel supplemented with granulated electrode carbon as required for carbon content. The melts were made in a high frequency induction furnace using an unlined magnesia crucible of either 200 pounds or 10 pounds capacity.

40 The smaller heats were initially charged. Furnace 45 heats larger than 10 pounds were slagged after the initial melt-down. For these heats, both the standard ferrochromium and nitrogen bearing ferrochromium were used, the nitrogen bearing ferrochromium being added after the standard grade.

45 Deoxidation was made with either an 80% Ni-20% Mg or MgFeSi (7% Mg-42% Si) alloy, or both, depending upon the quality of the alloy intended. Ferroalloy additions were then made as desired. The melts 50 were poured immediately into either cast iron or dry sand molds.

55 Analytical data on an alloy produced from a 10 pound heat, without slagging, and on a 100 pound heat, with slagging, are set out in Table I below. The alloys were 60 produced as sound castings and, as-cast, were feebly magnetic. On reheating to 2200° F., followed by air cooling, the magnetism disappeared completely, indicating a completely austenitic structure. The material from the 100 pound ingot was hot swaged and appeared to have 65 excellent hot working properties.

TABLE I  
*Compositions (percent) of cast alloys*

| Cr    | C    | N    | Mn   | S     | P     | Ni   | Mo   | Si   | Magnetic Response |                    |
|-------|------|------|------|-------|-------|------|------|------|-------------------|--------------------|
|       |      |      |      |       |       |      |      |      | As Cast           | 2,200° F.—air Cool |
| 20.81 | 0.46 | .23  | 0.83 | .010  | .014  | 0.72 | 0.01 | 0.75 | Very weak.....    | None.              |
| 21.05 | 0.65 | .29  | 0.86 | .013  | .024  | 0.64 | 0.01 | 0.87 | Weak.....         | Do.                |
| 21.15 | 0.35 | 0.38 | 0.86 | 0.018 | 0.017 | 0.02 | 0.01 | 1.17 | Strong.....       | Very weak.         |
| 20.60 | 0.52 | .32  | 1.02 | .011  | .023  | 0.59 | 0.02 | 0.82 | Mild.....         | None.              |
| 20.88 | 0.56 | .33  | 0.85 | .024  | .012  | 0.64 | 0.05 | 0.94 | Medium.....       | Do.                |
| 20.81 | 0.46 | .23  | 0.83 | .010  | .014  | 0.72 | 0.01 | 0.75 | Very weak.....    | Do.                |
| 21.05 | 0.65 | .29  | 0.86 | .013  | .024  | 0.64 | 0.01 | 0.87 | Weak.....         | Do.                |
| 23.98 | 0.36 | .29  | 0.77 | .014  | .026  | 0.13 | 0.01 | 0.61 | Strong.....       | Do.                |
| 26.28 | 0.46 | .33  | 0.84 | .019  | .014  | 0.40 | 0.01 | 0.68 | do.....           |                    |

Analytical data on wrought alloys produced by the above procedure are set out in Table II below.

We claim:

A process for the production of essentially austenitic

TABLE II

*Compositions (percent) of wrought alloys and phases present after quenching from 2200° F.*

| Si   | Mn   | S     | P     | C    | Ni   | Cr    | N     | Phases            |
|------|------|-------|-------|------|------|-------|-------|-------------------|
| 0.68 | 0.82 | 0.013 | 0.010 | 0.38 | 0.55 | 24.58 | 0.392 | Austenitic.       |
| 0.82 | 0.86 | 0.017 | 0.014 | 0.33 | 0.71 | 27.57 | 0.538 | Do.               |
| 1.01 | 0.98 | 0.010 | 0.012 | 0.47 | 0.25 | 26.55 | 0.260 | F-A. <sup>1</sup> |
| 1.15 | 0.98 | 0.010 | 0.008 | 0.47 | 0.25 | 26.89 | 0.587 | Austenitic.       |

<sup>1</sup> A stands for austenite and F for ferrite.

The physical properties of the new austenitic iron-chromium-carbon nitrogen alloys reveal distinctive characteristics of potential value in a range of industrial applications. Similar to the iron-manganese-carbon Hadfield steels, the chromium alloys show extreme work hardening. This effect is reflected in their resistance both to cutting and to deformation in the tensile test. Even though this austenite shows a hardness value of only about 20 Rockwell C, it is virtually impossible to cut it with ordinary tool steels although the materials can be cut readily with carbide tools. However, when the alloys are decomposed to ferrite, carbides and nitrides, they can be machined readily with ordinary cutting tools. The alloys then can be restored to the austenitic structure by reheating to greater than 2000° F. and cooling.

In the tensile test, very little localized necking occurs even though reduction of area values of 50 percent are attained. The tensile strength of a 27% chromium-0.5% carbon-0.7% nitrogen alloy is 138,000 p.s.i. The yield strength 90,000 p.s.i. The alloys, of course, are non-magnetic when in the completely austenitic state. In general the new alloys have value in corrosive environments, particularly at the higher chromium contents, where strength and abrasion resistance are required. The new alloys as such may not be well adapted for use at elevated temperatures since they tend to decompose to ferrite, carbides, and nitrides above about 800 to 900° F. The alloys can be beneficially modified in this respect by the introduction of additional alloying elements, for example, manganese, molybdenum, copper, nickel, cobalt, titanium, or aluminum. In slow bend tests, the austenitic alloys show a desirable degree of flexibility for mechanical shaping operations.

35 stainless steel alloys substantially free of ferrite without incorporating austenitizing amounts of metals effective therefor such as nickel, manganese, and the like which comprises forming a melt consisting essentially of about 21 to 33% chromium, about 0.2 to 1.0% carbon and an amount of nitrogen added in stably combined form in the range of 0.3 to 1.0% sufficient to maintain the relative proportions of nitrogen to carbon for any particular chromium content above the line in the phase diagram of the accompanying drawing, the balance of the 40 melt being iron except for incidental impurities, casting the resulting melt, rapidly cooling the cast product to a temperature below about 800° F., and thereafter refining the structure of the resulting alloy product by reheating to a temperature in the range of about 900 to 1300° F. 45 to decompose the alloy to a mixed phase product, thereupon heating to about 2000° to 2400° F. to reaustenitize the product, and finally rapidly cooling the reaustenitized alloy to below about 800° F.

55 References Cited in the file of this patent

UNITED STATES PATENTS

- 1,990,589 Franks \_\_\_\_\_ Feb. 12, 1935  
2,454,020 Weitzenkorn \_\_\_\_\_ Nov. 16, 1948  
2,657,130 Jennings \_\_\_\_\_ Oct. 27, 1953

60 OTHER REFERENCES

Monypenny: "Stainless Iron and Steel," second edition, London, Chapman & Hall Ltd., 1931, page 503.

65 Colbeck et al.: Journal of the Iron and Steel Institute, vol. 139, No. 1, 1939. Pages 99P-136P.